

May 25, 1937.

M. L. WADE

2,081,518

LOWERED POUR POINT OF OIL

Filed Sept. 4. 1934



INVENTOR.  
Maurer L. Wade

BY *Philip Lubkow*  
ATTORNEY.

## UNITED STATES PATENT OFFICE

2,081,518

## LOWERED POUR POINT OF OIL

Maner L. Wade, Long Beach, Calif., assignor to  
 Union Oil Company of California, Los Angeles,  
 Calif., a corporation of California

Application September 4, 1934, Serial No. 742,625

5 Claims. (Cl. 87—9)

This invention relates to the production of low pour point lubricating oil and to pour point depressing agents as compositions of matter.

One of the desirable characteristics of a high grade lubricating oil is a low pour point, i. e. a low temperature at which the oil congeals or ceases to flow. The pour point of an oil is measured according to the method specified by the American Society of Testing Materials D—97—30.

In the production of lubricating oils from waxy fractions it is customary at the present time to remove a substantial quantity of the wax from the oil in order that the final product will have a low pour point. This is usually accomplished by adding a suitable diluent such as naphtha to the waxy oil, chilling the mixture to a temperature sufficiently low to precipitate the wax and then removing the wax from the chilled mixture by settling, centrifuging or filtering. This operation is not only expensive but removes from the oil constituents which have a high lubricating oil value. Most waxes contained in lubricating oil fractions are characterized by a flat viscosity temperature slope, i. e. they have a low viscosity 20 gravity constant as measured by the method prescribed by Hill and Coates in the Journal of Industrial and Engineering Chemistry, volume 20, page 641 for 1928.

Oils which contain wax have a lower viscosity 30 gravity constant than that of the oil itself after the wax has been removed. Therefore where it is desired to produce oils of the lowest viscosity gravity constant it is undesirable to remove the wax from the oil.

Furthermore the separation of the wax from wax bearing oil results in a lower yield of the finished oil. The removal of the wax amounts to an appreciable lowering of the yield and furthermore an additional loss is occasioned by the oil 40 which is contained in the wax removed from the oil.

I have discovered a method of lowering the pour point of oil wherein it is unnecessary to remove all of the wax from the oil. I have discovered certain agents or materials, which, when added in relatively small amounts to oils having a high pour point, cause a substantial lowering of the pour point of the oil.

I have discovered that Montan wax is an effective pour point depressant for oils which have a high pour point. When a small quantity of Montan wax is added to an oil having a high pour point the pour point of this mixture is substantially lowered. For example a Santa Fe 55 Springs waxy distillate having a pour point of

50° F. was mixed with 0.3% of refined Montan wax and the pour point of this mixture or blend was found to be 10.0° F.

Montan wax occurs in lignite and is extracted therefrom by means of volatile solvents. Refined Montan wax has a melting point (Ubbelohde) between 80° and 86° C., an acid number of 64.0 and a saponification number of 67.0.

Crude or unrefined Montan wax may also be advantageously employed to lower the pour point 10 of oil. However this material is not as effective as the refined product. Crude Montan wax has a melting point of about 84° C. (Ubbelohde), an acid number of 26 and a saponification number of 92.0.

It is therefore an object of this invention to lower or depress the pour point of oil by the use of Montan wax.

I have also discovered that mixtures of certain materials are more effective for lowering the 20 pour point of oil than the respective materials comprising the mixture.

It is therefore an object of this invention to produce pour point depression agents comprising 25 mixtures of materials which conjointly are effective in lowering the pour point of oil.

It is another object of this invention to produce pour point depression agents from mixtures of materials which individually do not lower the pour point of oil to as great a degree as the 30 respective mixtures.

It is a further object of this invention to lower the pour point of lubricating oil by the addition of a material to said oil comprising a plurality of materials which in admixture with the oil cause 35 a substantial lowering of the pour point of the oil.

It is another object of this invention to produce relatively low pour point lubricating oil 40 from oil having a relatively high pour point which comprises adding to said high pour point oil a mixture of materials which conjointly are effective in lowering the pour point of said oil.

It is another object of this invention to lower the pour point of oil by the addition to said oil 45 of a mixture of materials which individually have little or no pour point depressing effect upon said oil but which in admixture cause a substantial lowering of the pour point of said oil.

The following table shows the pour point depressing qualities or characteristics of certain materials when added to a high pour point lubricating oil fraction and the pour point depressing qualities or characteristics of mixtures of these materials when added to the high pour point oil. 50 55

The oil used in conjunction with the pour point depression agents shown in this table is a Santa Fe Springs distillate having a pour point of 75 as shown in Test 1 of this table.

5 *Table*

| 10 | Test | Pour point depressant weight % added to the oil        | Pour point of the oil blended with the depressant °F. |
|----|------|--------------------------------------------------------|-------------------------------------------------------|
| 15 | 1    | None                                                   | 75                                                    |
|    | 2    | 0.5% condensation product                              | 70                                                    |
|    | 3    | 0.25% condensation product + 0.25% refined Montan wax  | 5                                                     |
|    | 4    | 1.0% of an extract from cracked petroleum pitch        | 65                                                    |
|    | 5    | + 0.5% refined Montan wax                              | 10                                                    |
|    | 6    | 1.0% of a cracked distillate                           | 60                                                    |
|    | 7    | 0.5% cracked distillate + 0.5% refined Montan wax      | 20                                                    |
| 20 | 8    | 1.0% I. G. E. wax                                      | 65                                                    |
|    | 9    | 0.5% cracked distillate + 0.5% I. G. E. wax            | 30                                                    |
|    | 10   | 0.3% I. G. O. P. wax                                   | 55                                                    |
|    | 11   | 0.15% condensation product + 0.15% I. G. O. P. wax     | 15                                                    |
|    | 12   | 0.3% I. G. B. wax                                      | 45                                                    |
|    | 13   | 0.15% condensation product + 0.15% I. G. B. wax        | 15                                                    |
| 25 | 14   | 0.3% I. G. S. wax                                      | 75                                                    |
|    | 15   | 0.15% condensation product + 0.15% I. G. S. wax        | 10                                                    |
|    | 16   | 0.30% ester gum                                        | 75                                                    |
|    | 17   | 0.15% condensation product + 0.15% ester gum           | 60                                                    |
|    | 18   | 0.30% stearic acid                                     | 75                                                    |
| 30 | 19   | 0.15% condensation product, + 0.15% stearic acid       | 20                                                    |
|    | 20   | 0.30% copal                                            | 75                                                    |
|    | 21   | 0.15% copal + 0.15% condensation product               | 65                                                    |
|    | 22   | 0.30% condensation product                             | 75                                                    |
|    | 23   | 1.0% polymerization product                            | 75                                                    |
|    | 24   | 0.6% polymerization product + 0.15% refined Montan wax | 20                                                    |
| 35 | 25   | 1.0% acetone extract from wax                          | 70                                                    |
|    | 26   | 0.5% Montan wax + 0.5% acetone extract from wax        | 35                                                    |
|    | 27   | 0.3% Carnauba wax                                      | 60                                                    |
|    | 28   | 0.15% Carnauba wax + 0.15% condensation product        | 15                                                    |
|    | 29   | 0.50% Montan wax                                       | 40                                                    |

40 The condensation product shown in Tests 2, 3, 11, 13, 15, 17, 19, 21, 22, and 28 of the above table is a condensation product made by the reaction of anhydrous aluminum chloride upon a 45 mixture of chlorinated paraffin wax and an aromatic hydrocarbon and is described in U. S. Patent No. 1,963,917. Therefore when I employ the term "condensation product" in the specification and claims I am referring to materials produced by the Friedel-Craft synthesis which are produced according to the process described in the aforementioned patent.

45 The cracked petroleum extract shown in Tests 4 and 5 of the above table was made by topping 55 a cracked asphaltic residue to 55% bottoms and a melting point (Ball and Ring) of 314° F. and then extracting these bottoms at ordinary temperature with naphtha to dissolve the oil-like bodies and precipitate the black or asphaltic 60 bodies. The fractions dissolved in the naphtha are then recovered by distilling the naphtha from the solution. It may also be prepared by extracting the asphaltic bottoms with light lubricating oil and decanting the lubricating oil solution away 65 from the black residue.

65 The cracked distillate employed in Tests 6 and 7 of the above table was made from a cracked asphaltic residue which had previously been topped to 65% overhead and 35% bottoms. The 70 bottom fraction had a melting point of about 325° to 350° F. (Ball and Ring). The 35% bottoms were distilled and the overhead fractions recovered from this material were employed in the manner shown in the above table under Tests 75 6 and 7. The overhead fractions from the 35%

bottoms has a melting point (Ball and Ring) of 198° F.

The I. G. waxes employed in Tests 8 to 15 inclusive of the above table are those described by Dr. Justin-Mueller of the I. G. Farbenindustrie Aktiengesellschaft in the November, 1931, issue of the "La Revue General de Teinture, Impression, Blanchiment et Appret". These products are also described on page 559 of the December 4, 1931, issue of the Chemical Trade Journal. These waxes are products of esterification of montanic alcohols with montanic acids. The montanic acids (which are high fatty acids with a high melting point) are obtained by the oxidation of the hydrocarbons in lignite, while the montanic alcohols are made by the reduction of the corresponding acids under a high pressure. Therefore, when I employ the term "products of esterification of montanic alcohols with montanic acids" in the specification and claims, I am referring to the above described materials produced as described in the aforementioned articles.

15 The wax employed in Tests 8 and 9 of the above table and denoted therein as the I. G. E. wax, has an acid number of 14.3, a saponification number of 142, a melting point (Ubbelohde) of 166° F., a specific gravity of 1.01-1.02, an esterification index of 140-155, and contains about 20 7 to 10% of unsaponifiables.

25 The wax employed in Tests 10 and 11 of the above table, and denoted therein as the I. G. O. P. wax, has an acid number of 13.8, a saponification number of 113, a melting point (Ubbelohde) of 219° F., specific gravity of 1.03-1.04, an esterification index of 90-120 and a 7 to 10% content 30 of unsaponifiable materials.

35 The wax employed in Tests 12 and 13 of the above table and denoted therein as "I. G. B." wax has an acid number of 57.8, a saponification number of 148, a melting point (Ubbelohde) of 177.5° F., specific gravity 0.98, an esterification index of 125 to 135 and a 22% content of unsaponifiable materials.

40 The wax employed in Tests 14 and 15 of the above table has an acid number of 143, a saponification number of 170, a melting point (Ubbelohde) of 181° F., a specific gravity of 1.01-1.02 and an 8 to 10% content of unsaponifiables.

45 The ester gum shown in Tests 16 and 17 is a glyceride produced by the reaction of rosin (abietic acid) upon glycerin. It is a solid varying from light amber to brown in color.

50 The copal shown in Tests 21 and 22 of the above table is a fossil resin containing free fatty acids and esters.

55 The polymerization product shown in Tests 23 and 24 of the above table is a synthetic oil having the following characteristics:

|                                     |      |    |
|-------------------------------------|------|----|
| Gravity A. P. I. at 60° F.          | 22.0 | 60 |
| Viscosity, Saybolt universal at 210 |      |    |
| seconds                             | 687  |    |
| Flash, °F. (Cleveland open cup)     | 390  |    |
| Fire, °F. (Cleveland open cup)      | 460  |    |
| Pour point, °F.                     | 30.0 |    |
| Conradson carbon value, percent     | 0.39 | 65 |
| Acid number                         | 0.47 |    |
| Saponification number               | 72.0 |    |

70 This material is made from vegetable and mineral oil and is fully described in Kohlenwasserstofföle und Fette by D. Holde, 7th edition at page 372. According to the description by Holde the aforementioned polymerization product is prepared by the blow discharge of a mineral or fatty oil, the process, through ionic discharge, causing a forma- 75

tion of polymerization products of high molecular weight, as well as of a very high viscosity. Therefore when I employ the term "polymerization product" in the specification and claims I am referring to the materials produced according to the description of Holde in Kohlenwasserstofföle und Fette, 7th edition, at page 372.

The acid numbers and saponification numbers of the materials shown in this specification were obtained according to the American Society of Testing Material methods D-188-27T and D-94-28 respectively.

The acetone extract shown in Tests 25 and 26 of the above table is the acetone soluble portion of wax. Untreated Santa Fe Springs wax distillate was diluted with liquid propane, chilled and filtered. The wax cake recovered was then extracted with acetone and the acetone and dissolved fractions were separated from the undissolved material. The acetone solution was distilled to remove the acetone and the extract recovered was employed as shown in Tests 25 and 26 of the above table.

From an inspection of the data in the table it will be noted that the mixtures of materials are more effective for lowering the pour point of oil than the individual materials.

For example condensation product mixed with Montan wax, products of esterification of montanic alcohol with montanic acids, ester gum, stearic acid, copal or polymerization product is more effective in lowering the pour point of oil than any of the single members of this group.

Furthermore it will be noted from the table that a mixture of cracked distillate and a product of esterification of montanic acid with montanic alcohol is more effective for lowering the pour point of lubricating oil than either cracked distillate or a product of esterification of montanic acid with montanic alcohol (Tests 6, 8, and 9); extract from cracked petroleum pitch mixed with Montan wax is more effective than the cracked extract alone (Tests 4 and 5); cracked distillate mixed with Montan wax is more effective than cracked distillate alone (Tests 6 and 7); and acetone extract from wax mixed with Montan wax is more effective than the wax extract alone (Tests 25 and 26).

Furthermore from Tests 22, 27, and 28 it will be seen that a mixture of carnauba wax and condensation product is decidedly more effective in lowering the pour point of the oil than either condensation product or carnauba wax.

The above examples are merely illustrative and are not to be construed as limitations upon the invention which I claim.

The effect of mixed pour point depression agents or modifiers upon the pour point of lubricating oil is also shown in Graphs A, B, and C of Figure 1. The ordinate of this figure shows the pour point of the oil and the abscissa shows the composition of the mixed pour point depressant added to the oil. Graphs A, B, and C show the effect of adding 0.15%, 0.30%, and 0.45% respectively of a mixed pour point depressant containing condensation product and Montan wax in the respective proportions shown on the ordinate.

From an inspection of the data presented in Fig. 1 it will be noted that the original oil had a pour point of 75° F. As will be seen from Graph A the addition of 0.15% of condensation product lowered the pour point of this oil to 70° F.; the addition to the oil of 0.15% of a mixture of Montan wax and condensation product containing 25% Montan wax and 75% condensation

product lowered the pour point of the oil to 45° F.; the addition of 0.15% of a mixture of Montan wax and condensation product containing 35% Montan wax and 65% condensation product lowered the pour point of the oil to 20° F.; the addition of 0.15% of a mixture of Montan wax and condensation product containing 75% Montan wax and condensation product lowered the pour point of the oil to 20° F.; and, the addition of 0.15% Montan wax to the oil lowered the pour point to 10° F. From this graph it is apparent that mixtures of condensation product and Montan wax are more effective than either of these materials. Furthermore it will be noted that 0.15% of this mixed modifier is most effective when the proportion of Montan wax contained in the mixture lies between the proportions of 25% and 75%.

The data presented on Graph B shows the effect of adding 0.30% of a mixture of condensation product and Montan wax upon the pour point of the oil. From this graph it will be noted that this mixture is most effective for lowering the pour point of the oil when the proportion of Montan wax contained in the mixture lies between 50% and 75%.

The data presented in Graph C shows the effect of adding 0.45% of a mixture of condensation product and Montan wax upon the pour point of the oil. From this graph it will be seen that this mixture is most effective for lowering the pour point of the oil when the proportion of Montan wax contained in the mixture lies between 25% and 75%.

From an inspection of Graphs A, B, and C of the figure it will also be noted that increasing amounts of these mixed pour point depressants added to the oil produces an increase in the lowering of the pour point of the oil.

From a consideration of the data presented in the figure it is seen that eutectic mixtures are obtained between the wax, condensation product and Montan wax. Furthermore it is seen from this figure that the pour point of the eutectic mixture depends upon the relationship between the quantities of the respective depressants contained in the mixture and that there is an optimum range of proportions within which these pour point depression agents must exist in the oil in order to obtain maximum lowering of the pour point. For example the optimum range for the mixture shown on Graph A exists when the proportion of Montan wax contained in the mixture lies between 25% and 75% or the amount of condensation product contained in the mixture lies between 25% and 75%. The "eutectoids" formed with the waxy oil and the mixture containing proportions of Montan wax and condensation product within these limits have the lowest pour points which can be produced by mixing the waxy oil with condensation product and Montan wax.

The lowest pour point "eutectoids" to be obtained in the mixtures shown on Graph B will exist when the Montan wax or condensation product contained in the Montan wax-condensation product mixture constitutes from 50% to 75% of the mixture. Furthermore the lowest pour point "eutectoids" to be obtained in the mixtures shown on Graph C will be when the Montan wax or condensation product constitutes from 25% to 75% of the mixed depressant. By the term "eutectoid" I mean oil and wax mixed with a plurality of pour point depressing agents compounded in such proportions

as to produce a product which exhibits a minimum pour point.

The above example of eutectic mixtures of oil, wax, Montan wax and condensation product 5 (shown in the figure) is only one example of this phenomena, however I do not wish to limit myself by this example as the other mixed depressants shown in the table form similar "eutectoids" as those shown in Graphs A, B, and C.

10 It is therefore an object of this invention to add a plurality of pour point depressing agents to waxy oil in amounts sufficient to produce a eutectic mixture having a minimum pour point.

The pour point depression agents produced according to this invention have been found to be 15 more effective in lowering the pour point of oil containing wax of the crystalline type than upon oils containing wax of the ceresin type. The crystalline waxes are usually found in overhead 20 distillates and are characterized by relatively low melting points.

I claim:

1. A composition of matter comprising a wax bearing mineral oil blended with 0.15% to 0.45% 25 of a mixture of Montan wax and a condensation product obtained by reacting an aromatic hydrocarbon with a chlorinated aliphatic hydrocarbon in the presence of a metallic halide of the Friedel-Craft catalyst type.

30 2. A composition of matter comprising, a wax bearing mineral oil blended with about 0.15% to 0.25% of a condensation product obtained by reacting an aromatic hydrocarbon with a chlorinated aliphatic hydrocarbon in the presence of

a metallic halide of the Friedel-Craft catalyst type and blended with one of the members selected from the group consisting of a montanic alcohol ester of montanic acid, carnauba wax, copal and Montan wax, said composition of matter 5 being fluid at ordinary atmospheric temperature.

3. A composition of matter comprising a wax bearing mineral oil blended with 0.15% to 0.50% of Montan wax and with a small quantity of one of the members selected from the group consisting of cracked petroleum pitch, extract from cracked pitch, cracked petroleum distillate, a condensation product obtained by reacting an aromatic hydrocarbon with a chlorinated aliphatic hydrocarbon in the presence of a metallic 15 halide of the Friedel-Craft catalyst type, and a polymerization product obtained by volatilization of vegetable and mineral oil, said composition of matter being fluid at ordinary atmospheric temperature.

4. A composition of matter comprising a wax bearing mineral oil blended with about 1.0% of a mixture of Montan wax and an extract obtained from cracked petroleum pitch.

5. A composition of matter comprising a wax 25 bearing mineral oil blended with about 0.3% of a mixture of a condensation product obtained by reacting an aromatic hydrocarbon with a chlorinated aliphatic hydrocarbon in the presence of a metallic halide of the Friedel-Craft 30 catalyst type and an ester of montanic alcohol and montanic acid.

MANER L. WADE.